

Feb. 6, 1962

J. V. ROBINSON ET AL

3,020,176

CAST COATED PAPER AND METHOD OF MAKING THE SAME

Filed March 13, 1958



FIG. 1

INVENTORS  
JAMES V. ROBINSON,  
BY EARL B. BROOKBANK, JR.

*James V. Robinson*  
ATTORNEYS

1

3,020,176

## CAST COATED PAPER AND METHOD OF MAKING THE SAME

James V. Robinson and Earl B. Brookbank, Jr., Chillicothe, Ohio, assignors to The Mead Corporation, Dayton, Ohio, a corporation of Ohio

Filed Mar. 13, 1958, Ser. No. 721,106

18 Claims. (Cl. 117—64)

This invention relates to the production of high gloss cast surfaced mineral coated papers, and more particularly to agents which are effective in providing ready and complete release of such coated papers from a casting surface.

Various known methods of producing cast-surfaced mineral-coated papers are similar in that a wet and plastic coated paper is pressed into adherent contact with a finishing surface, such as a highly polished chromium plated drum or belt, and dried thereon, and thereafter the dried coated paper is intended to separate from the drum with a surface finish which is desirably a replica of the finishing surface. A difficulty heretofore encountered in the production of cast-surfaced mineral-coated paper is sticking of the dried and set coating to the finishing surface, resulting in marring of the coated paper surface by particles of the dried coating which adhere to the finishing surface. Indeed, this sticking may become so extreme that the entire area of the paper in contact with the finishing surface becomes tightly bonded thereto and is only removed by long and laborious treatment. Obviously, such a sticking condition makes the process of cast coating inoperable.

Several methods have been proposed to substantially overcome this sticking of mineral coatings to the finishing surface. For example, one such method seeks to maintain on the finishing surface an invisible film, substantially less than 2000 Angstrom units in thickness, of oil or other fatty material, such substances being designated as oleaginous film forming materials, which are characterized as relatively water-insoluble liquids which wet the casting surface and spread into a continuous film, yet will not vaporize too readily at operating temperatures. The coating on the web is intended to adhere firmly to the casting surface until the coating has dried to a non-plastic condition and is thereafter released from the casting surface. Satisfactory results utilizing this method allegedly are obtained only by periodic application of the oleaginous material directly to the casting surface, or, preferably, application of the oleaginous compound to the casting surface by incorporation of a quantity of the oleaginous release agent in the coating composition.

Obviously, this method is subject to the objection that the required function of oleaginous material on the casting surface is necessarily dependent on, and the exact quantity thereof determined by, a skilled operator who watches the point at which the paper leaves the casting surface, and hopefully increases or decreases the amount of oleaginous material on the chromium drum and/or in the coating composition in order to avoid sticking on the one hand, or loss of gloss in the finished paper on the other, the latter condition resulting from the use of an excess of oleaginous material. Even a moderate increase in the thickness of the oleaginous film may cause a mottled appearance of the finished coated paper and may leave sufficient grease on the surface of the coated paper both to make the paper distasteful to handle and to produce scumming on an offset printing press when the paper is subsequently printed.

An object of this invention is to provide for the continuous production of cast surfaced mineral coated paper whereby certain chemical release agents are utilized for facilitating ready release of coating material from a casting surface.

2

Another object of this invention is to provide an improved method for continuously producing cast surfaced mineral coated paper, which method facilitates ready release of coating from a casting surface.

5 Another object is to provide water-soluble non-ionic surface active materials which have the property of readily effecting separation of cast surfaced mineral coated paper from a casting surface on which it is dried.

It is a further object to provide such non-ionic surface active materials which are effective over a relatively wide range of concentrations.

Another object is to provide a method of the foregoing type adapted to relatively high speed production.

Numerous other objects of this invention will more fully hereinafter appear.

The sole figure of the drawing schematically illustrates one method of this invention.

The release agents, according to this invention, include certain water-soluble non-ionic surface active materials 20 which are either normally liquid at room temperature, or become liquid at the operating temperature of the casting surface (which temperature varies with particular operating conditions, but normally falls in the range of 170—230° F.). Such agents have been found to be especially 25 useful when added to the coagulant bath disclosed in co-pending application Serial No. 648,227, filed March 25, 1957 by John W. Smith, now U.S. Patent 2,950,214, and which is assigned to the same assignee as this application. According to the method therein disclosed for producing 30 cast surfaced mineral coated paper, an aqueous mineral coating composition comprising dispersed pigments and an adhesive is applied to a paper web in predetermined quantity and uniformly distributed thereon, and the coated surface of the web while still wet is thereafter contacted 35 with a coagulant bath whereby the adhesive component of the freshly applied mineral coating is converted into a gel, without substantial drying, in a manner so as to prevent undesirable distortion of the coating film. The gelled coating is thereafter pressed against a casting surface and dried thereon.

For example, reference is made to the accompanying drawing wherein a paper web 11 to be coated is drawn from a supply roll 10 of suitable paper base stock and is led over guide rolls 12 and 13 to pass through the 45 apparatus in the color applying zone. The web 11 passes through the nip of the coating application rolls 14, 15 where a predetermined amount of coating suspension is applied thereto and distributed with sufficient uniformity over the web surface to give the desired weight 50 of coating material per unit area on the web.

The coating color is fed through a suitable supply line and by suitable means to one or more discharge pipes or nozzles 23 and into the nip between rolls 15 and 24 which have the direction of rotation as indicated, the color forming a pool 25. Doctor 26, as shown, functions to maintain the pool in the nip between rolls 15 and 24 and any well known doctoring means may be employed.

The coated web is then brought with the coated side 60 out tightly around roll 16 which dips into the coagulant and release agent bath of this invention contained in a tub 17. The coated paper 11 is then transferred by press roll 18, after the coating has been formed into a non-tacky tough deformable gel, into nip 19, and thereby 65 into contact with a heated finishing roll 20 having a smooth casting surface. The web 11 remains in contact with casting roll 20 until the coating spontaneously releases after it has substantially completely dried and is removed by tension roll 21 to winder roll 22.

Various coating materials as described in the copending application, supra, may be employed in practicing the present invention and as indicated by the formulations

hereinafter set forth, the coating material generally comprises a mineral and an adhesive in aqueous medium.

A color formula which has been found to function satisfactorily in the practicing of the invention is of the following composition, wherein the parts by weight are taken on a dry basis:

*Example I*

|                                                                                                   | Parts by weight |
|---------------------------------------------------------------------------------------------------|-----------------|
| Clay (English coating clay)                                                                       | 42.0            |
| Calcium carbonate                                                                                 | 42.0            |
| Casein (Argentina)                                                                                | 12.0            |
| Caustic soda (parts per 100 parts of casein)                                                      | 6.0             |
| Sodium pyrophosphate                                                                              | 0.75            |
| Calcium stearate                                                                                  | 0.5             |
| Dow 512-R latex (butadiene-styrene copolymer 30:70)                                               | 6.0             |
| Di-isobutylphenoxyethoxyethylbenzyl-ammomiumchloride, monohydrate (Hyamine 1622, Rohm & Haas Co.) | 0.05            |

Such color gives satisfactory results in the practicing of this invention when admixed with water to have a solids content of approximately 50.5%.

The following examples of color formulations which have likewise been used satisfactorily are set forth for purposes of illustration, but not of limitation. The parts by weight of these compositions are taken on a dry basis:

*Example II*

|                                                  | Parts by weight |
|--------------------------------------------------|-----------------|
| Clay (English coating clay)                      | 42.0            |
| Calcium carbonate                                | 42.0            |
| Soya protein (refined)                           | 12.0            |
| Ammonia-26° Bé. (parts per 100 parts of protein) | 12.0            |
| Dow 512-R latex                                  | 4.0             |
| Sodium pyrophosphate                             | 0.75            |
| Calcium stearate                                 | 0.5             |
| Hyamine 1622                                     | 0.05            |

*Example III*

|                                                  |      |
|--------------------------------------------------|------|
| Clay (English coating clay)                      | 38.0 |
| Calcium carbonate                                | 41.0 |
| Satin white                                      | 5.0  |
| Alpha protein                                    | 12.0 |
| Ammonia-26° Bé. (parts per 100 parts of protein) | 12.0 |
| Dow 512-R latex                                  | 4.0  |
| Sodium pyrophosphate                             | 0.75 |
| Calcium stearate                                 | 0.5  |
| Lignasan                                         | 0.05 |

*Example IV*

|                                                       |      |
|-------------------------------------------------------|------|
| Clay (English coating clay)                           | 51.0 |
| Calcium carbonate                                     | 30.0 |
| Alpha protein                                         | 18.0 |
| Azite(dicyandiamide) (parts per 100 parts of protein) | 25.0 |
| Ammonia-26° Bé. (parts per 100 parts of protein)      | 12.0 |
| Sodium pyrophosphate                                  | 0.75 |
| Calcium stearate                                      | 0.5  |
| Lignasan                                              | 0.05 |

*Example V*

|                                                  |      |
|--------------------------------------------------|------|
| Calcium carbonate                                | 84.0 |
| Alpha protein                                    | 12.0 |
| Ammonia-26° Bé. (parts per 100 parts of protein) | 18.0 |
| Dow 512-R latex                                  | 4.0  |
| Sodium pyrophosphate                             | 0.75 |
| Calcium stearate                                 | 0.5  |
| Hyamine 1622                                     | 0.05 |

*Example VI*

|                                                       |      |
|-------------------------------------------------------|------|
| Clay (domestic coating clay)                          | 81.0 |
| Soya protein (refined)                                | 12.0 |
| Azite(dicyandiamide) (parts per 100 parts of protein) | 25.0 |
| Ammonia-26° Bé. (parts per 100 parts of protein)      | 15.0 |
| Sodium pyrophosphate                                  | 0.75 |
| Sulphonated tallow (Vegetol)                          | 1.0  |
| Calcium stearate                                      | 0.5  |
| Dow 512-R latex                                       | 7.0  |
| Hyamine 1622                                          | 0.1  |

As described in the copending application, supra, the conversion of the adhesive component of the coating to the gel state is almost instantaneous, requiring only a fraction of a second following initial contact with the coagulant. And mixing of the release agent of this invention with the coating composition is greatly restricted, and occurs to only a minor extent. Thus, the release agent is carried on the surface of the gelled coating as a liquid solution (which also contains the coagulant salts) to the casting nip. A small quantity of this solution passes through the casting nip, together with the gelled coating, as a fluid film thereon, and is dried in contact with the casting surface, whereby the release agent is concentrated at the plane of release, and functions to provide clean separation of the cast coated web from the casting surface. Accordingly, incorporation of the water-soluble non-ionic surface active release agents of this invention in the aforesaid coagulant bath insures the presence of the release agent at the point where needed to provide the desired function. Cast coated webs so prepared carry coatings which are relatively free from contamination by release agents, the amount of such agent appearing in the cast coated paper being of the order of 0.0007 to 0.10 lb. per 1000 sq. ft., depending on operating conditions and on the concentration of the agent used in the coagulant bath which normally ranges from 0.125 to 5.0% by weight, this in turn depending on the particular release agent employed.

While not wishing to be restricted thereby, it is believed that the mechanism by which such water-soluble non-ionic surface active materials operate to provide release is concerned with the deposition of a very thin film of a liquid between the casting surface and the surface of the dried coating, and that such a film, being of low cohesive strength, splits with one part remaining on the paper and the other part remaining on the casting surface. According to this mechanism, the film of release agent between the coating and the casting surface does not come into existence until all or nearly all of the water present has been evaporated. Thus, good contact and/or adherence of the wet, plastic coating to the casting surface is obtained, a condition desirable for attainment of a truly cast surface of gloss approaching that of the casting surface, but evaporation of the water which sets the coating to a non-plastic state also serves to form a releasing film of liquid at the location and at the time it is required to bring about release of the dried coating from the casting surface. This action is relatively independent of the amount of release agent present, providing only that there is a sufficient amount to form the releasing film as the water evaporates.

When following the teachings of this invention, the wet, plastic, gelled coating adheres to the casting surface when pressed thereon, and there is little or no apparent relative movement of the coating and the casting surface until the coating has been dried. The coating, after drying, is readily, completely and cleanly separated from the casting surface presumably because of the splitting of the thin layer of liquid film deposited or formed between the coating and casting surface during the drying operation.

Since this invention provides for the formation of the

releasing liquid film at the time and place of release from the casting surface, it is relatively free from a major limitation inherent in the use of the prior art oily or so-called oleaginous materials, in that the presence of an excess over the minimum required to provide ready release does not cause a loss of gloss in the cast-surfaced mineral coated paper, as is the case with said oleaginous materials.

In the development of this invention, it was discovered that a great number of water soluble non-ionic surfactants could be employed as suitable release agents. For example, materials such as water soluble reaction products of phenols, alcohols, higher fatty acids, amides, amines, propylene oxide, and/or ethylene oxide were found to be especially suitable. By water soluble surfactants are meant those surfactants which are self-dispersible in water and yield non-settling suspensions or clear solutions in water. Such surfactants in the practice of this invention when incorporated with coagulating electrolyte solutions, as for example, calcium formate, retain their characteristics of solubility or suspension stability with no perceptible change.

While preferred water soluble non-ionic surfactants for the purpose of this invention are selected from the class comprising polymers of ethylene oxide and/or propylene oxide and their simple ethers, equally good results were obtained with agents selected from the following chemical classes of non-ionic surface active agents: polymers of ethylene oxide and/or propylene oxide and their simple ethers; esters of polyoxyethylene; polyethanolamine-fatty acid condensates; polyoxyethylene thio ethers; polyoxyethylene phenol ethers; substituted fatty amides; and polyoxyethylene amides.

A considerable number of the non-ionic water soluble surfactants of this invention are liquids or pastes at room temperature, but as mentioned hereinbefore, some of the effective materials are normally solid at room temperature, but melt and become liquid at or below the temperature of the casting surface, so that their function cannot be distinguished from that of the products which are normally liquids at room temperature.

The invention will be more clearly understood by reference to the following examples, which serve to illustrate but not limit the scope of this invention.

In each of the examples set forth hereinafter, a typical coating composition, comprising dispersed mineral pigments and an adhesive in aqueous medium was applied to a paper web in predetermined amount and spread to a uniform, smooth film thereon, as set forth and diagrammatically shown in the copending application, supra. The wet, coated web, without substantial drying, was then contacted on its coated side with a coagulating solution of 5% calcium formate which also contained one of the water soluble release agents of this invention. The web traveled to and was pressed against a highly polished chromium plated, heated casting drum, whereby a considerable portion of the coagulant and release surfactant which was carried on the surface of the web was squeezed from the surface by the action of the casting nip, which permitted only a relatively thin film of said solution to pass through on the surface of the gelled coating. Heat supplied to the interior of the drum, as by steam, evaporated the water from the gelled coating and from the layer of solution lying between the coating and the casting surface. In each case, the coated web, after reaching substantial dryness, separated easily and completely from the casting surface, and was observed to have a gloss closely approaching that of the polished casting surface. And except for the inclusion of the relatively water soluble release surfactants of this invention in the coagulating bath, the preferred procedure and apparatus used in the practice of this invention is the same as that disclosed in the referred to co-pending application, supra.

The following listing presents specific examples of commercially available water soluble, non-ionic surfactants, in the concentration set forth, which were used in the practice of this invention to effect the desirable release as described hereinbefore.

| Example | Trade-name                       | Composition                                       | Concentration of Release Agent in Coagulant Solution |
|---------|----------------------------------|---------------------------------------------------|------------------------------------------------------|
| 10      | Ucon 50HB 100                    | polyoxyethylene mono-alkyl ether.                 | 1.0                                                  |
| 15      | do                               | do                                                | 0.5                                                  |
| 3       | do                               | do                                                | 0.25                                                 |
| 4       | Ucon 50HB 2000                   | do                                                | 1.0                                                  |
| 5       | do                               | do                                                | 0.5                                                  |
| 6       | Pluronic F-68                    | Polyoxyethylene ether of polyoxypropylene.        | 1.0                                                  |
| 7       | do                               | do                                                | 0.5                                                  |
| 20      | Tergitol XH                      | polyoxyethylene glycol ether.                     | 1.0                                                  |
| 9       | Tergitol XD                      | polyoxyethylene glycol                            | 1.0                                                  |
| 10      | Carbowax 200                     | (M. W. 200).                                      | 1.0                                                  |
| 11      | Carbowax 600                     | polyoxyethylene glycol (M. W. 600).               | 1.0                                                  |
| 25      | Carbowax 1000                    | polyoxyethylene glycol (M. W. 1000).              | 1.0                                                  |
| 13      | Carbowax 6000                    | polyoxyethylene glycol (M. W. 6000).              | 0.5                                                  |
| 14      | Carbowax 20M                     | polyoxyethylene glycol (M. W. 20,000).            | 0.5                                                  |
| 15      | Methoxypolyethylene Glycol       | methoxypolyethylene glycol.                       | 1.0                                                  |
| 30      | Polypropylene Glycol (M. W. 150) | polypropylene glycol (M. W. 150).                 | 1.0                                                  |
| 16      | Polypropylene Glycol (M. W. 425) | polypropylene glycol (M. W. 425).                 | 1.0                                                  |
| 17      | Ethofat 142/60                   | mono red oil fatty acid ester of polyoxyethylene. | 1.0                                                  |
| 18      | do                               | do                                                | 0.5                                                  |
| 35      | Ethofat 242/25                   | mono rosin fatty acid ester of polyoxyethylene.   | 1.0                                                  |
| 21      | Sterox CD                        | tall oil fatty acid ester of polyoxyethylene.     | 1.0                                                  |
| 22      | Nonisol 210                      | oleic acid ester of polyoxyethylene.              | 5.0                                                  |
| 40      | Nonisol 300                      | stearic acid ester of polyoxyethylene.            | 5.0                                                  |
| 23      | Nonisol 100                      | lauric acid ester of polyoxyethylene.             | 5.0                                                  |
| 25      | Tween 80                         | polyoxyethylene sorbitan mono-oleate.             | 1.0                                                  |
| 26      | do                               | do                                                | 0.5                                                  |
| 27      | do                               | do                                                | 0.25                                                 |
| 28      | Cerfak N-100                     | polyethanolamine-fatty acid condensate.           | 1.0                                                  |
| 29      | Alrosol B                        | fatty alkylo amide condensate.                    | 1.0                                                  |
| 30      | Ninol 737                        | fatty acid alkanol amide.                         | 5.0                                                  |
| 50      | Nonic 234                        | polyethylene glycol tert. dodecyl thioether.      | 1.0                                                  |
| 32      | Nonic 218                        | do                                                | 1.0                                                  |
| 33      | Nonic 260                        | do                                                | 1.0                                                  |
| 34      | Polytergent G-300                | alkyl phenol polyglycol ether.                    | 1.0                                                  |
| 55      | do                               | do                                                | 0.5                                                  |
| 36      | Igepal CA 630                    | iso-octylphenoxypolyoxyethylene ethanol.          | 1.0                                                  |
| 37      | Michelene DDS                    | alkyl amido alcohol.                              | 1.0                                                  |
| 38      | do                               | do                                                | 5.0                                                  |
| 39      | Michelene DLD                    | fatty acid amide ester.                           | 5.0                                                  |
| 40      | Antarox G-100                    | alkyl polyoxyethylene ethanol amide.              | 5.0                                                  |
| 60      |                                  |                                                   |                                                      |

All of the release agents in the above examples were found to be unaffected when used in combination with an electrolyte solution such as the electrolyte solution utilized for coagulation of the adhesive component of the coating mix. While the above stated examples were prepared in connection with a 5% calcium formate solution as the coagulant, the use of other electrolytes, such as calcium acetate, zinc acetate, calcium lactate, aluminum sulfate, and the like does not interfere with the proper functioning of the release agents of this invention.

Since the methods and products herein described are for the purpose of illustration only, it is to be understood that the present invention includes all modifications and

equivalents which fall within the scope of the invention which is defined by the appended claims.

What is claimed is:

1. In the manufacture of cast-surfaced mineral coated paper, the steps comprising coagulating the coating while still mobile and fluent and deformable on the paper by direct contact with a coagulating electrolyte to form said coating into a tough deformable gel, concomitantly incorporating a water-soluble non-ionic surfactant with said coagulating electrolyte which imparts substantially complete separation of said coating from a casting surface, and thereafter bringing said coating into contact with a casting surface, said surfactant being liquid on said casting surface and imparting substantially complete separation of said coating from said casting surface.

2. In the manufacture of cast-surfaced mineral coated paper, the steps comprising coagulating the coating while still mobile and fluent and deformable on the paper by direct contact with a coagulating electrolyte to form said coating into a tough deformable gel, concomitantly incorporating a water-soluble non-ionic surfactant with said coagulating electrolyte which imparts substantially complete separation of said coating from a casting surface, said surfactant being selected from the group consisting of water-soluble: polymers of ethylene and propylene oxide and their simple ethers, esters of polyoxyethylene, polyethanolamine-fatty acid condensates, polyoxyethylene thio ethers, polyoxyethylene phenol ethers, substituted fatty amides and polyoxyethylene amides, and thereafter bringing said coating into contact with a casting surface, said surfactant being liquid on said casting surface and imparting substantially complete separation of said coating from said casting surface.

3. The process of producing a cast-surfaced mineral coated paper in accordance with claim 2 wherein the surfactant consists essentially of water-soluble polymers of ethylene oxide and their simple ethers.

4. The process of producing a cast-surfaced mineral coated paper in accordance with claim 2 wherein the surfactant consists essentially of water-soluble polymers of ethylene oxide and propylene oxide.

5. The process of producing a cast-surfaced mineral coated paper in accordance with claim 2 wherein the surfactant consists essentially of water-soluble esters of polyoxethylene.

6. The process of producing a cast-surfaced mineral coated paper in accordance with claim 2 wherein the surfactant consists essentially of water-soluble polyoxyethylene phenol esters.

ylene phenol esters.

7. The process of producing a cast-surfaced mineral coated paper in accordance with claim 2 wherein the surfactant consists essentially of water-soluble polyoxyethylene boron esters of fatty acids.

8. In the manufacture of cast-surfaced mineral coated paper, the steps comprising coagulating the coating while still mobile and fluent and deformable on the paper by direct contact with a coagulating electrolyte to form said coating into a tough deformable gel, concomitantly incorporating a non-ionic water-soluble surfactant with said coagulating electrolyte which imparts substantially complete separation of said coating from a casting surface, said surfactant being selected from the water-soluble reaction products of phenols, alcohols, higher fatty acids, amides, amines, mercaptans and propylene oxide respectively with ethylene oxide, and thereafter bringing said coating into contact with a casting surface, said surfactant being liquid on said casting surface and imparting substantially complete separation of said coating from said casting surface.

9. The process of producing a cast-surfaced mineral coated paper in accordance with claim 8 wherein the surfactant consists essentially of a water-soluble reaction product of ethylene oxide.

product of ethylene oxide.

10. The process of producing a cast-surfaced mineral coated paper in accordance with claim 8 wherein the sur-

factant consists essentially of a water-soluble reaction product of ethylene oxide and propylene oxide

11. The process of producing a cast-surfaced mineral coated paper in accordance with claim 8 wherein the surfactant consists essentially of a water-soluble reaction product of ethylene oxide and alcohols.

12. The process of producing a cast-surfaced mineral coated paper in accordance with claim 8 wherein the surfactant consists essentially of a water-soluble reaction product of ethylene oxide and fatty acids.

13. The process of producing a cast-surfaced mineral coated paper in accordance with claim 8 wherein the surfactant consists essentially of a water-soluble reaction product of ethylene oxide and hexitan esters.

14. The process of producing a cast-surfaced mineral coated paper in accordance with claim 8 wherein the surfactant consists essentially of a water-soluble reaction product of ethylene oxide and a phenol.

15. In the manufacture of cast-surfaced mineral coated

15. In the manufacture of cast-surfaced mineral coated  
20 paper, the steps comprising coagulating the coating while  
still mobile and fluent and deformable on the paper by  
direct contact with a coagulating electrolyte to form said  
coating into a tough deformable gel, concomitantly in-  
corporating a water-soluble non-ionic surfactant with said  
25 coagulating electrolyte which imparts substantially com-  
plete separation of said coating from a casting surface,  
the concentration of said surfactant in the coagulating  
electrolyte being of the order of 0.25 to 5.0%, and there-  
after bringing said coating into contact with a casting sur-  
30 face, said surfactant being liquid on said casting surface  
and imparting substantially complete separation of said  
coating from said casting surface.

16. In the manufacture of cast-surfaced mineral coated paper, the steps comprising coagulating the coating while

35 still mobile and fluent and deformable on the paper by direct contact with a coagulating electrolyte to form said coating into a tough deformable gel, concomitantly incorporating a water-soluble non-ionic surfactant with said

40 incorporating a water-soluble high-ionic surfactant with said coagulating electrolyte which imparts substantially complete separation of said coating from a casting surface, said surfactant being selected from the group consisting of water-soluble: polymers of ethylene and propylene ox-

45 soluble polymers of ethylene and propylene oxide and their simple ethers, esters of polyoxyethylene, polyethanolamine-fatty acid condensates, polyoxyethylene thio ethers, polyoxyethylene phenol ethers, substituted fatty amides and polyoxyethylene amides, the concen-

50 fatty amides and polyoxyethylene amides, the concentration of said surfactant in the coagulating electrolyte being of the order of 0.25 to 5.0%, and thereafter bringing said coating into contact with a casting surface, said surfactant being liquid on said casting surface and imparting substantially complete separation of said coating from said casting surface.

17. In the manufacture of cast-surfaced mineral coated paper, the steps comprising coagulating the coating while still mobile and fluent and deformable on the paper by direct contact with a coagulating electrolyte to form said

direct contact with a coagulating electrolyte to form said coating into a tough deformable gel, concomitantly incorporating a non-ionic water-soluble surfactant with said coagulating electrolyte which imparts substantially complete separation of said coating from a casting surface.

60 plie separation of said coating from a casting surface, said surfactant being selected from the water-soluble reaction products of phenols, alcohols, higher fatty acids, amides, amines, mercaptans and propylene oxide respectively with ethylene oxide, the concentration of the water-

65 tively with ethylene oxide, the concentration of the water-soluble reaction product in the coagulating electrolyte being of the order of 0.25 to 5.0%, and thereafter bringing said coating into contact with a casting surface, said surfactant being liquid on said casting surface and imparting substantially complete separation of said coating from

70 said casting surface.

18. A cast surfaced mineral coated paper substantially identical with the product obtainable by the process of claim 1.

## References Cited in the file of this patent

## UNITED STATES PATENTS

|           |                |                |           |
|-----------|----------------|----------------|-----------|
| 2,674,619 | Lunsted        | Apr. 6, 1954   | 2,769,725 |
| 2,718,509 | Lunsted et al. | Sept. 20, 1955 | 2,773,114 |
| 2,730,531 | Payne et al.   | Jan. 10, 1956  | 2,776,226 |
|           |                |                | 2,819,184 |
|           |                |                | 2,835,653 |

|              |              |
|--------------|--------------|
| Hart         | Nov. 6, 1956 |
| McAuslan     | Dec. 4, 1956 |
| Hart         | Jan. 1, 1957 |
| Smith et al. | Jan. 7, 1958 |
| Haas et al.  | May 20, 1958 |